



US005665509A

**United States Patent [19]****Brantly****[11] Patent Number: 5,665,509****[45] Date of Patent: Sep. 9, 1997****[54] ELECTROPHOTOGRAPHIC CARRIER COMPOSITIONS HAVING IMPROVED LIFE****[75] Inventor: Thomas Brantly, Nashua, N.H.****[73] Assignee: Nashua Corporation, Nashua, N.H.****[21] Appl. No.: 748,377****[22] Filed: Nov. 13, 1996****[51] Int. Cl.<sup>6</sup> G03G 9/113****[52] U.S. Cl. 430/108; 430/137; 430/106.6****[58] Field of Search 430/108, 137****[56] References Cited****U.S. PATENT DOCUMENTS**

|            |         |                 |           |
|------------|---------|-----------------|-----------|
| Re. 32,883 | 3/1989  | Lu              | 430/110   |
| 4,286,038  | 8/1981  | Lu et al.       | 430/108   |
| 4,298,672  | 11/1981 | Lu              | 430/108   |
| 4,433,040  | 2/1984  | Niimura et al.  | 430/109   |
| 4,614,700  | 9/1986  | Yamamoto et al. | 430/122   |
| 4,868,082  | 9/1989  | Kohri et al.    | 430/106.6 |
| 4,883,736  | 11/1989 | Hoffend et al.  | 430/110   |
| 4,935,326  | 6/1990  | Creatura et al. | 430/108   |

|           |         |                  |           |
|-----------|---------|------------------|-----------|
| 5,071,725 | 12/1991 | Kubo et al.      | 430/108   |
| 5,071,726 | 12/1991 | Maniar           | 430/106.6 |
| 5,104,762 | 4/1992  | Shirose et al.   | 430/106.6 |
| 5,126,225 | 6/1992  | Wilson et al.    | 430/108   |
| 5,192,635 | 3/1993  | Inukai et al.    | 430/108   |
| 5,230,980 | 7/1993  | Maniar           | 430/137   |
| 5,393,631 | 2/1995  | Horikoshi et al. | 430/108   |
| 5,411,832 | 5/1995  | Yoerger          | 430/108   |
| 5,491,044 | 2/1996  | Wilson et al.    | 430/110   |

**FOREIGN PATENT DOCUMENTS**

|          |        |       |         |
|----------|--------|-------|---------|
| 64-29861 | 1/1989 | Japan | 430/108 |
| 64-29866 | 1/1989 | Japan | 430/108 |

*Primary Examiner*—Roland Martin  
*Attorney, Agent, or Firm*—Weingarten, Schurgin, Gagnebin & Hayes LLP

**[57]****ABSTRACT**

Electrophotographic carrier compositions comprising a coating containing a resin and a mixture of positive and negative charge agents, and methods for making such carriers; and electrophotographic developers containing the same are disclosed.

**16 Claims, No Drawings**

## ELECTROPHOTOGRAPHIC CARRIER COMPOSITIONS HAVING IMPROVED LIFE

### FIELD OF THE INVENTION

This invention relates to electrophotographic carrier compositions in general, and in particular, to carrier compositions having a coating which provides for longer life and less carrier scum than conventional carriers, and for electrophotographic developers containing these carriers.

### BACKGROUND OF THE INVENTION

Electrophotographic processes and apparatus employ the use of toners, which are generally comprised of a resin and a colorant, along with other desirable additives like charge control agents. In general, a desired image is formed on an organic photoconductor (OPC) coated medium such as a drum or belt in the form of a charged pattern representing the image. Toner is then electrically attracted to the charge on the drum and adheres to the drum in an imagewise manner. Lastly, the toner image is transferred from the OPC medium to an image-receiving substrate (typically paper) and fused, resulting in permanent image formation on the substrate.

In magnetic brush development systems, charge is imparted to the toner triboelectrically by mixing toner particles with carrier particles, which are typically resin-coated steel particles about 20 to 200 $\mu$  in diameter. The toner particles adhere to the oppositely-charged carrier particles and are conveyed from a hopper to the magnetic brush roller system. On the roller chains of the toner-laden carrier particles form, and as the chains are conveyed on the roller into the gap between the roller and the OPC medium, the charged toner particles are attracted to and deposited on the oppositely-charged latent image areas of the OPC medium. The carrier particles are collected and recycled for remixing with toner.

Since the carrier is a recyclable component of the developer, it is naturally of great concern to make it last as long as possible so as to minimize cost. A persistent problem in the art is "toner scum", wherein after a period of mixing with toner, toner particles irreversibly adhere to the carrier, rendering triboelectric charging ineffective and necessitating replacement of the carrier.

A related problem is the selection of coatings for the carrier particles. When designing developer for copying machines, many factors must be considered, one of which is the triboelectric characteristics of the carrier particles vis-a-vis the particular toner required by the copier mechanics. Much development work is devoted to toner chemistry and physics and the goal of having the toner form a good printed image on the paper. However, because the toner cannot form an image on the photoconductor unless the toner is sufficiently triboelectrically charged, then subsequently separated from the carrier particles during imaging (within the mechanical and physical copier design parameters chosen), the chemical and physical design of the carrier must be considered also. Therefore, carrier and toner must be engineered to work together as a developer. When many different developer formulations are under development, for many different machines, this can be a complicated effort. It would therefore be preferable to be able to formulate and characterize one carrier formulation that can be easily and predictably optimized to the particular demands of any given toner and its respective copying system, so as to produce a "tailor-made" developer at a lower cost.

Another issue that arises in toner manufacture is that of unremoved solvent such as methyl ethyl ketone (MEK) in

the carrier coating after the carrier has been processed. Trace amounts of solvent in the carrier coating are deleterious to developer performance because toner can adhere to carrier particles having unremoved MEK. Furthermore, the MEK will dissolve the toner, creating a sticky residue on the surface of the carrier that greatly reduces the triboelectric effectiveness of the carrier.

### SUMMARY OF THE INVENTION

- 10 The present invention relates to carrier compositions having a coating providing longer carrier life and less carrier scum than those used in conventional developer systems, as well as electrophotographic developers containing these carriers. A carrier composition as presently disclosed comprises a core material and a coating comprising a resin, and a mixture of positive and negative charge agents. The triboelectric characteristics of the coating may be adjusted by varying the ratio of positive to negative charge agents in the coating so as to adjust the net charge on the carrier particles to a desired value. In one advantageous embodiment the coating composition comprises a fluoropolymers resin and a mixture of Nigrosine; and chromate (1-) bis{3-hydroxy-4-[2-hydroxy-(3,5-dinitrophenyl) azo]-N-phenyl-2-naphthalene carboxamato(2-)}-hydrogen ("TRH") or salts thereof.
- 15

### DETAILED DESCRIPTION OF THE INVENTION

A carrier coating as presently disclosed comprises a resin and a mixture of positive and negative charge agents is disclosed which provides a carrier material having longer life. Additionally, a carrier coating is disclosed having desirable triboelectric characteristics which may be predictably obtained by adjusting the ratio of the positive and negative charge agents in the coating so as to adjust the net charge on the carrier particles to a desired value. The combination of resin and certain charge agents also provides the surprising advantage of allowing for the easier removal of solvents such as MEK used in coating the core particles.

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5240

5245

5250

5255

5260

5265

5270

5275

5280

5285

5290

5295

5300

5305

5310

5315

5320

5325

5330

5335

5340

5345

5350

5355

5360

5365

5370

5375

5380

5385

5390

5395

5400

5405

5410

5415

5420

5425

5430

5435

5440

5445

5450

5455

5460

5465

5470

5475

5480

5485

5490

5495

5500

5505

5510

5515

5520

dinium halides such as cetyl pyridinium halide; organic sulfate or sulfonates; distearyl dimethyl ammonium sulfate; bisulfates; and dioxazines.

Negative charge agents that may be used include heliogen green pigment; metal complexes of phthalic acid, naphthoic acid, or salicylic acid; copper-phthalocyanines; perylenes; quinacridones;  $\alpha$ -fluorobenzoic acids;  $p$ -halo phenyl carboxylic acids; azo pigments; metal-salt azo pigments; azo-chromium complexes; chromate (1-) bis{3-hydroxy-4-[(2-hydroxy-3,5-dinitrophenyl) azo]N-phenyl-2-naphthalene carboxamato(2-)}-hydrogen ("TRH") or salts thereof.

An important distinction of the carrier compositions disclosed herein is that the charge agents are incorporated in the carrier coating, compared to the usual practice of dispersing such agents in toner or developer. The direct benefits of the invention, e.g., reduction of toner scum, are obtained as a result. The charge agents may be added to the carrier coating in any effective amount so as to obtain the benefits disclosed in this patent application, but not so much as to deteriorate the other requirements of carrier materials, e.g., abrasion resistance and proper charging characteristics. Keeping this in mind, the charge agents may be desirably added in a range from about 0.5 to 10% by weight, based on the total weight of the dry coating.

Other indirect and unexpected benefits, however, are also obtained, such as the simplification of the task of manufacturing carrier for a wide range of copying or development systems. For example, since the triboelectric properties of the carrier may be varied predictably by changing the proportion of positive to negative charge agents in the coating, it is contemplated that one apparatus, comprising storage and metering means for resin, positive, and negative charge agent; and a mixing apparatus is all that is needed for one to produce carrier core coating. One needing to make carrier for a particular system would simply need to do no more than determine the proportions of each of the coating components necessary for the proper triboelectric characteristics, i.e., determine the desired net charge on the carrier particles, enter in the proper settings on the equipment to dispense the proper amounts of each component, mix and prepare the coating, and coat the core particles in the usual manner.

It has also been noted that solvent such as MEK used as a carrier solvent to enable the coating to be sprayed on the core particles surprisingly, can be more easily removed when the coating contains charge agents such as Nigrosine. When conventional coatings are made, i.e., without the presently disclosed charge agents, the drying procedure requires much care to ensure that all of the solvent is removed from the carrier particles at the maximum temperature allowable by the coating. However, the presently described coatings comprising charge agents such as Nigrosine allow the carrier to be dried at a higher allowable temperature, better ensuring that all of the coating solvent is removed and avoiding the undesired result of toner sticking to the carrier when blended as developer.

Toner that may be used with carrier as described herein essentially comprises a thermoplastic binder consisting of a thermoplastic resin or mixture of resins, and colorants such as carbon black, finely dispersed dye pigments, or soluble dyes, and may further include infra-red or ultra-violet absorbing substances and substances that produce black in admixture. Suitable resins include transparent thermoplastic resins such as polyesters, polyethylenes, polystyrenes and copolymers thereof such as styrene-acrylic resin and styrene-butadiene resin; (meth)acrylates; polyvinyl chlo-

rides; vinyl acetates; copoly(vinyl chloride-vinyl acetate);, copoly(vinyl chloride-vinyl acetate-maleic acid); vinyl butyryl resins; polyvinyl alcohols; polyurethanes; polyamides; polyolefins; and styrene polymer. The diameter of dry toner particles for use in magnetic brush development typically ranges from about 8 to 13 $\mu$ , with an average of about 10 $\mu$  in general-purpose applications. For high resolution development, the toner particle diameter is typically in the 3 to 8 $\mu$  range.

"Electrophotographic printing" is defined herein to include both electrographic and electrophotographic printing. (As used herein, the term "electrophotographic" also includes the direct image-wise application of electrostatic charges on an insulating support, for example by ionography.) In electrographic printing, an electrostatic charge is deposited imagewise on a dielectric recording member. In electrophotographic printing, an overall electrostatically charged photoconductive dielectric recording member is image-wise exposed to conductivity increasing radiation producing thereby a "charge area" or "discharge area" toner-developable charge pattern on the recording member.

The following non-limiting example illustrates a specific embodiment of the invention.

#### EXAMPLE 1

A carrier composition in accordance with the disclosure was made as follows. A coating solution was prepared by first making a dispersion concentrate and then diluting the concentrate for coating. The concentrate was prepared by dissolving 40.0 g Oxy-461 fluoropolymer (Occidental Petroleum) in 150 g methyl ethyl ketone (MEK); combining this solution with 5.0 g Vulcan 9A32 (Cabot Corporation) carbon black, 2.5 g Nigrosine Base B (Orient Chemical) and 2.5 g TRH (Hodogaya Chemical); and milling the mixture in a laboratory attritor for 40 minutes. The attritor was cooled with running water and had  $\frac{1}{8}$ " steel shot for a milling medium. A replicate concentrate was prepared, added to the first concentrate and then the total solids reduced to 8% with MEK.

The solution was then spray coated onto 5000 g of Anchor Steel 100/150 steel shot heated to 120° F. in a laboratory size fluid bed coater. When the coating operation was completed, the coating was further dried for one hour at 125° F.

The carrier was blended with toner and placed in a copier for testing. The developer was used to make one million copies. It had a charge-to-mass ratio of 15.2  $\mu$ C/g at 4.6% toner concentration throughout the test run. All the copies made were high quality images with solid area densities ranging from 1.36 to 1.49.

#### EXAMPLE 2

A comparative test was conducted to show the beneficial effects of a carrier composition made accordance with the disclosure versus a control. The test procedure was as follows. The developer (comprising toner and carrier) was added to a photocopier machine to make copies. At certain intervals the developer was sampled to conduct surface fluorine measurements on the carrier by ESCA. Q/m and TC (toner concentration) were measured by the blowoff method. The stability of the surface fluorine, Q/m and TC values over time is a measurement of how well the developer stabilizes and "breaks in" in the machine; these values should stabilize after an initial refractory period, allowing for acceptable experimental variations. Both carriers were made generally according to the procedure in Example I, with a coat weight

of 2% (i.e., weight of the coating based on the total weight of carrier plus coating). The carrier compositions were I (control): Oxy-461 fluoropolymer/carbon black/Nigrosine Base B (85/10/5), and II (invention): Oxy-461 fluoropolymer/carbon black/Nigrosine Base B/TRH (80/10/5/5).

The data are shown in Tables 1 and 2. It can be seen that developer in accordance with the disclosure remains desirably stable over several hundred copies, in comparison to the other developer tested.

TABLE 1

| Copies<br>( $\times 1000$ ) | F<br>(%) | Q/m<br>(uC/g) | TC<br>(%) |
|-----------------------------|----------|---------------|-----------|
| 0                           | 31.7     | 17.4          | 2.9       |
| 40                          | 12.6     | 11.1          | 1.8       |
| 50                          | 14.3     | 11.8          | 1.8       |
| 105                         | 11.3     | 10.9          | 1.6       |
| 125                         | 10.2     | 11.8          | 1.5       |
| 155                         | 11.5     | 11.8          | 1.4       |
| 459                         | —        | 14.3          | 1.2       |

TABLE 2

| Copies<br>( $\times 1000$ ) | F<br>(%) | Q/m<br>(uC/g) | TC<br>(%) |
|-----------------------------|----------|---------------|-----------|
| 0                           | 34.2     | 10.5          | 3.6       |
| 30                          | 15.6     | 11.3          | 2.3       |
| 50                          | 17.3     | 13.8          | 4.0       |
| 100                         | 16.5     | 15.6          | 4.2       |
| 150                         | 15.9     | 15.8          | 4.4       |
| 200                         | 16.0     | 14.6          | 4.8       |
| 500                         | 16.6     | 15.6          | 4.4       |
| 750                         | 15.9     | 16.7          | 3.9       |
| 950                         | 18.4     | 13.7          | 4.8       |

The foregoing description is meant to be illustrative of novel carrier compositions, electrophotographic developers containing the same, and methods of making improved carriers and developers. Other embodiments and variations will be apparent to those of ordinary skill in the art without departing from the inventive concepts contained herein. Accordingly, this invention is to be viewed as embracing each and every novel feature and novel combination of features present in or possessed by the invention disclosed herein and is to be viewed as limited solely by the scope and spirit of the appended claims.

What is claimed is:

1. An electrophotographic carrier composition, comprising carrier particles comprising a core and a coating thereupon, said coating comprising a resin and a mixture of positive and negative charge agents.

2. The carrier composition of claim 1 wherein said positive charge agent is selected from the group consisting of Nigrosine dyes; triamino triphenylmethanes; cationic dyes; alkyl pyridinium halides; organic sulfates or sulfonates; distearyl dimethyl ammonium sulfate; bisulfates; dioxazines; and mixtures thereof.

3. The carrier composition of claim 1 wherein said negative charge agent is selected from the group consisting of heliogen green pigment; metal complexes of phthalic acid, naphthoic acid, or salicylic acid; copper-phthalocyanines; perylenes; quinacridones; o-fluorobenzoic acids; p-halo phenyl carboxylic acids; azo pigments; metal-salt azo pigments; azochromium complexes; chromate (1-) bis{3-hydroxy-4-[(2-hydroxy-3,5-dinitrophenyl) azo]-N-phenyl-2-naphthalene carboxamato(2-)}-hydrogen or salts thereof; and mixtures thereof.

4. The carrier composition of claim 1 wherein said resin is selected from the group consisting of chlorotrifluoroethylene vinylidene fluoride; polyvinylidene fluoride; polytrifluoroethylene; polytetrafluoroethylene; polycarbonates; cellulose acetate butyrate; substituted or unsubstituted polyvinyl pyrrolidones; glass; polysulfones; acrylonitrile-butadiene-styrene terpolymer; polyesters; phenolic resins; nylons; alkyl celluloses; polymethylmethacrylate (PMMA); polystyrenes; polyisobutylenes; natural rubbers; polyformaldehyde; polyamides; polyurethanes; styrene-acrylonitrile copolymers; styrene-butadiene copolymers; and mixtures thereof.

5. The carrier composition of claim 1 wherein said resin is a fluoropolymeric resin; said positive charge agent is a Nigrosine dye; and said negative charge agent is chromate (1-) bis{3-hydroxy-4-[(2-hydroxy-3,5-dinitrophenyl) azo]-N-phenyl-2-naphthalene carboxamato(2-)}-hydrogen ("TRH") or a salt thereof.

6. The carrier composition of claim 1 wherein the average particle size of said core is in the range of 20 to 200 $\mu$ .

7. The carrier composition of claim 1 wherein said mixture of positive and negative charge agents is present in said coating in an amount of from about 0.5 to 10% by weight, based on the total weight of the dry coating.

8. An electrophotographic developer composition, comprising carrier particles comprising a core and a coating thereupon, said coating comprising a resin and a mixture of positive and negative charge agents; and toner particles.

9. The developer composition of claim 8 wherein said positive charge agent is selected from the group consisting of Nigrosine dyes; triamino triphenylmethanes; cationic dyes; alkyl pyridinium halides; organic sulfates or sulfonates; distearyl dimethyl ammonium sulfate; bisulfates; dioxazines; and mixtures thereof.

10. The developer composition of claim 8 wherein said negative charge agent is selected from the group consisting of heliogen green pigment; metal complexes of phthalic acid, naphthoic acid, or salicylic acid; copper-phthalocyanines; perylenes; quinacridones; o-fluorobenzoic acids; p-halo phenyl carboxylic acids; azo pigments; metal-salt azo pigments; azochromium complexes; chromate (1-) bis{3-hydroxy-4-[(2-hydroxy-3,5-dinitrophenyl) azo]-N-phenyl-2-naphthalene carboxamato(2-)}-hydrogen or salts thereof; and mixtures thereof.

11. The developer composition of claim 8 wherein said resin is selected from the group consisting of chlorotrifluoroethylene vinylidene fluoride; polyvinylidene fluoride; polytrifluoroethylene; polytetrafluoroethylene; polycarbonates; cellulose acetate butyrate; substituted or unsubstituted polyvinyl pyrrolidones; glass; polysulfones; acrylonitrile-butadiene-styrene terpolymer; polyesters; phenolic resins; nylons; alkyl celluloses; polymethylmethacrylate (PMMA); polystyrenes; polyisobutylenes; natural rubbers; polyformaldehyde; polyamides; polyurethanes; styrene-acrylonitrile copolymers; styrene-butadiene copolymers; and mixtures thereof.

12. The developer composition of claim 8 wherein said resin is a fluoropolymeric resin; said positive charge agent is a Nigrosine dye; and said negative charge agent is chromate (1-) bis{3-hydroxy-4-[(2-hydroxy-3,5-dinitrophenyl) azo]-N-phenyl-2-naphthalene carboxamato(2-)}-hydrogen ("TRH") or a salt thereof.

13. The developer composition of claim 8 wherein the average particle size of said core is in the range of 20 to 200 $\mu$ .

14. The developer composition of claim 8 wherein said mixture of positive and negative charge agents is present in

said coating in an amount of from about 0.5 to 10% by weight, based on the total weight of the dry coating.

15. The developer composition of claim 8 wherein said toner particles have a diameter from about 8 to 13 $\mu$ .

16. A method of adjusting the triboelectric characteristics of a carrier composition containing a core and a resin-containing coating, comprising the step of preparing a coating material for application to metal core particles

comprising resin and positive and negative charge agents, wherein said ratio of said positive and negative charge agents is effective to impart a desired net charge to said carrier particles, and the step of applying said coating material to a metal core.

\* \* \* \* \*